

## UNITED STATES PATENT OFFICE.

FRANCIS I. DU PONT AND ERNEST DU PONT, OF WILMINGTON, DELAWARE, ASSIGNEES,  
BY MESNE ASSIGNMENTS, TO U. S. F. POWDER COMPANY, OF WILMINGTON, DELA-  
WARE, A CORPORATION OF DELAWARE.

## SMOKELESS EXPLOSIVE POWDER AND PROCESS OF MAKING SAME.

No Drawing. Original application filed January 24, 1919, Serial No. 272,857. Divided and this application filed April 24, 1920, Serial No. 376,287. Renewed January 24, 1921, Serial No. 439,689. This application filed August 8, 1921. Serial No. 490,728.

This invention relates to flashless powders and processes of producing the same, and it comprises a powder having an accelerating rate of combustion of such a nature, as to 5 deliver muzzle gases not igniting in contact with air, such powder comprising a cellular body or matrix of colloided nitrocellulose containing included solid particles adapted to produce corresponding open cells or cavities 10 during the combustion of the powder; and it further comprises a method of producing such a powder wherein nitrocellulose is intimately admixed with solid particles of black powder, or of an oxygen-evolving, 15 combustion-quickeners material, such as a mixture of potassium nitrate and barium nitrate, and colloided to produce a honeycomb structure with the admixed solids in the cells, etc., all as more fully hereinafter set 20 forth and as claimed.

The object of our invention is to produce a smokeless explosive ordnance powder which, when used as a propellant charge in a gun, will approximately eliminate, or at least 25 very materially reduce, the muzzle flash; that is, light-emitting combustion or explosion beyond the muzzle. To accomplish this it is necessary that the powder should be substantially consumed and combustion actions over before the gaseous mass emerges 30 from the muzzle of the gun. It is not merely sufficient that the composition and structure of the powder should be such as to promote rapid accelerative burning, but it is also essential that this rapid burning should be effected without substantial increase of 35 chamber pressure in order thereby to avoid erosion of the gun barrel.

It is the usual practice to effect the burning of ordnance powder in a progressive way by forming perforations through the mass of a powder grain, so that the grains, which are rather large sized units requiring appreciable time for complete combustion, 45 will burn from the inside as well as from the outside, thus exposing to the flame, as the burning proceeds, a progressively increasing superficial area. There is a progressive acceleration of combustion.

50 The manufacture of smokeless explosives from nitrocellulose or pyroxylin is now an old art and such powders are usually "col-

loided"; a term used in the art to designate a treatment with solvents (usually acetone or ether-alcohol) to remove structure and convert the pyroxylin into an amorphous integral body. The solvents may be used in quantity sufficient to make a solution or in amount merely sufficient to plasticize; the final result being the same. These colloided smokeless powders are relatively slow burning and in order to accelerate combustion and produce a different pressure curve in the gun, it is usual to use them as perforated grains. Combustion on the walls widens 65 these perforations, offering a constantly increasing burning area. Conditions are ordinarily so adjusted as to cause a maximum rate of combustion just before the projectile leaves the muzzle. In the actions in a gun, 70 the work done on the projectile and gas expansion are heat-absorbing, while combustion is heat-developing; these balancing against each other. By postponing the maximum heat evolution in the way in which 75 it is done in these perforated powders, the gases leave the muzzle very hot. And as pyroxylin contains an excess of carbon, the muzzle gases are combustible, causing a secondary combustion or explosion with the aid 80 of air, this giving the flash.

We have discovered that the rate of progression acceleration of the burning in this type of powder may be substantially increased, without increase of chamber pressure, by distributing in a colloided mass of nitrocellulose powder a flame propagating agent which will carry the flame from the exposed surfaces, through a multitude of minute developed channels, into the interior. 90 of the powder grains, thereby bringing all the colloided nitrocellulose much more speedily into progressive contact with the fire and effecting an earlier complete consumption of the powder than is the case 95 where reliance is had solely upon relatively large and coarse mechanical perforations. In the present invention a different type of burning is superimposed on that resulting from these perforations.

100 It has been assumed that the flash or light produced at the muzzle of a gun is due to the fact that propellant powders composed substantially entirely of nitrocellulose have

an actual deficiency of oxygen below that which would be necessary to burn all of the carbon, and that minute particles of carbon, intensely heated, actually escape from the 5 muzzle of a gun and combine with the oxygen of the atmosphere in precisely the same way as do the particles of carbon in an ordinary jet of illuminating gas. In other words, there is a secondary combustion or 10 explosion beyond the muzzle; this giving the flash. While this may be a correct explanation of the phenomenon, we have found by prolonged experiment that in suppressing flash by the use of our agents in our 15 way, it is not essential that the ingredients added shall actually contain an excess of oxygen; that is, it is not necessary to try to burn the excess of carbon in the gun. In fact, we have used with equal success one 20 flame propagating agent having an excess of oxygen and another in which there is no oxygen available for the nitrocellulose, with an equal degree of success.

In the present invention, we superimpose 25 upon the old type of acceleration by the aid of perforations, another type resulting from progressively developing cavities in the grain; a sort of pitting action. In so doing, we are enabled to obtain a new type of combustion. And we have found that by proper regulation of the details of manufacture, we can produce a colloided pyroxylin powder which will develop satisfactory pressure curves in the gun, while at the same 30 time permitting the gases to leave the muzzle at a temperature at which, or in a condition in which, they will not ignite with the air. In other words, we do away with the secondary combustion or explosion which occurs beyond the muzzle with the ordinary 35 types of perforated, colloided nitrocellulose. In our new powder we usually employ the ordinary perforations and in addition give the colloided pyroxylin a cellular or honeycomb structure; the cells being filled with 40 solids adapted to cause quick local action and development of free cell walls adapted for free combustion.

If a particle or grain of a quicker-burning 45 explosive, such as black powder, be contained within a body of colloided nitrocellulose, when ignition reaches this grain, it disappears, leaving a pit or cavity in the nitrocellulose and then combustion follows 50 along the cavity walls. The effect is as if a new perforation had just been made at this point. The same result may be obtained by using crystals or particles of oxygen-evolving substances, such as a mixture of barium 55 nitrate and potassium nitrate. In a colloided nitrocellulose containing a particle of such a substance, when ignition reaches the 60 particle, there is a local evolution of oxygen which quickens combustion of the nitrocellulose lying next the particle, opening up

a space along the interface and giving the result of a newly developed pit or cavity. While the way in which the black powder and the oxidant act in developing pits or cavities is different in detail, the result is 70 the same; progressive opening of pits or cavities and avoidance of flash. With oxygen-evolving substances, if the amount employed be sufficient, the excess of carbon in the pyroxylin is consumed, giving muzzle 75 gases which will not burn.

In certain co-pending applications, we have described and claimed various powders and processes of making the same embodying the stated principles. In the application filed June 12, 1918, under Serial No. 239,531, we described and claimed the manufacture of a powder wherein pyroxylin was intimately admixed with fine ammonium nitrate and, sometimes, nitroglycerin; a 80 colloiding solvent being employed. As the colloiding solvent does not dissolve the ammonium nitrate, the result is a colloided or integralized mass of nitrocellulose containing distributed fine crystalline particles of ammonium nitrate. In another application, filed January 24, 1919, as Serial No. 272,857, of which the present application is a division, we described, as in the present case, a type of flashless powder made by first mixing nitrocellulose and either black 85 powder or a mixture of barium and potassium nitrate and afterwards colloiding, but restricted the claims to the use of such nitrates. In another application, originally filed February 23, 1921, as Serial No. 447- 90 229, we describe and claim another embodiment of the present invention wherein the specific flame propagating agent is a bichromate, or a mixture of a bichromate and carbon. In the present application, we describe and claim, in the specific claims, the use of black powder as a flame propagating 95 agent.

It is not sufficient that the added flame 100 propagating agent shall merely be effective to expedite the consumption of the nitrocellulose, but it must be such an agent as will do this without substantially increasing the chamber pressure, without seriously fouling the gun and without producing an excess of smoke. This not merely materially narrows the range of substances which would be otherwise available, but after the proper substances have been ascertained by experiment, the further problem arises of adding them in proper proportions to the nitrocellulose. Finally, after this information is acquired, the addition of the flame propagating agent to the nitrocellulose must precede any substantial colloiding of the nitrocellulose.

The characteristics of a fire propagating 110 agent such as black powder and of a fire propagating agent such as a mixture of

barium and potassium nitrates are, of course, quite dissimilar, the most notable difference being that the latter has an excess of oxygen, which it evolves when heated, while the former is a complete explosive and has no available oxygen.

Where a mixture of the two salts above named is used, we prefer to use about two parts of the barium salt to one part of the potassium salt, although these proportions may be varied. The total of the two ingredients should form about 8 to 12 per cent of the entire explosive. In no case should it exceed 20 per cent, while we distinctly prefer not to exceed 15 per cent. On the other hand, the proportion may be as low as 4 per cent and still very materially reduce the flash, although we prefer a minimum of about 7 or 8 per cent. The objection to using a large proportion of this fire propagating agent is that it results in objectionably fouling the gun, and moreover; a relatively large proportion produces no useful effect in the elimination of the flash, this being, for all practical purposes, attained by a relatively small proportion.

Where black powder is used as the flame propagating agent, we may use about the same proportion as above specified for the nitrates. A needlessly large proportion of black powder will produce an objectionable amount of smoke and should be carefully avoided. We prefer, therefore, to use as small a percentage of black powder as is possible, consistent with securing the desired results. As low as two per cent of black powder gives substantially flashless results and the black powder content may even be reduced to one-half of one per cent and still very materially reduce the flash.

Whether the flame propagating agent be one or the other of the above materials, or some equivalent substance, or combination of substances, the process of adding the agent to the nitrocellulose is of great importance. Unless the agent be so added as to effect a very thorough and intimate association of the particles, the finished powder will give non-uniform and uncertain results as a commercial product, in which uniformity and certainty of action are essential.

In carrying out our process it is necessary, in order to secure certain and uniform results, to thoroughly incorporate the flame propagating agent with the nitrocellulose before colloiding. We proceed by taking soluble nitrocellulose and add thereto the specified proportion of the flame producing agent, wet it with about thirty per cent of a suitable blending liquid, such as water or gasoline, and incorporate the same in a standard black powder wheel mill for about an hour or an hour and a quarter. The liquid added should be one which does not chemically combine with the explosive in-

gredients, or does not combine with them except to form a solution from which the solvent may be expelled by drying or by displacement otherwise. We prefer to use gasoline. Without the thorough moistening of the powder, the mixing operation, in any mill of the kind specified, would be attended with serious danger.

After the ingredients are thus thoroughly incorporated, the added liquid, or most of it, is expelled by drying or otherwise and then the colloiding agents, ether and alcohol, are added, and the entire mixture is thoroughly colloided in a kneading machine for about an hour. After the powder has been formed into grains of the usual type employed in ordnance, a considerable proportion of alcohol and ether is distilled off, a certain proportion remaining in the finished product.

The removal of the alcohol and ether should not be effected in any way which will cause removal of the fire carrying agent, as that would produce a certain undesirable porosity in the finished powder, whereas porosity, or porosity alone, is not the result desired, but rather a proper dissemination of the fire propagating agent through colloided nitrocellulose. The thorough incorporation of the ingredients is of the utmost importance, and it seems to be practically essential to first thoroughly incorporate the fire propagating agent with the nitrocellulose and afterward colloid; in other words, to rather closely adhere to the procedure above described.

The resultant powder is, to all intents and purposes, "flashless", there is no serious fouling of the gun, and the smoke produced is so limited in volume as to be unobjectionable.

If the colloiding agent be added at the beginning of the mixing operation, substantial incorporation of the nitrocellulose and the fire propagating agent will nevertheless occur before the colloiding action, and a flashless powder will be ultimately produced, but it is distinctly advantageous to add the colloiding agent after the operation of mixing the soluble nitrocellulose and fire propagating agent has been completed and after the expulsion of the liquid.

It should be clearly understood, however, that the colloiding of the nitrocellulose prior to the addition of the fire propagating agent would be, in substance, the addition of such agent to smokeless powder, and would be ineffective in accomplishing the purposes of our invention. Moreover, black powder, and various salts, have been added to certain so-called smokeless or semi-smokeless powders in other proportions and in other ways for other purposes.

In specifying a flame propagating agent we do not use the words to mean substances

which are only readily inflammable or combustible or even materials which might, when added to ingredients other than colloided nitrocellulose, render them combustible or increase their rate of bearing; but it is intended to be confined to substances which, contained in colloided nitrocellulose, will, by themselves, or in conjunction with such colloided nitrocellulose, increase the rate of burning of the explosives, as herein described, substantially beyond the rate of burning of colloided nitrocellulose alone.

We intend herein to claim the use of a flame propagating agent generically, and the use of black powder specifically; other pending applications hereinbefore recited being specific to certain other flame propagating agents.

Having now fully described our invention, what we claim and desire to protect by Letters Patent is.

1. The process of making "flashless" smokeless propellant powder with a progressively increasing rate of burning which comprises adding to and thoroughly incorporating with soluble nitrocellulose a flame propagating agent, and afterward completely colloiding with ether and alcohol and retaining the flame propagating agent in the finished explosive.

2. The process of making "flashless" smokeless propellant powder with a progressively increasing rate of burning which comprises adding to soluble nitrocellulose a flame propagating agent, moistening with a liquid adapted to be afterward expelled, thoroughly incorporating, expelling the added liquid, and afterward completely colloiding with ether and alcohol.

3. The process of making "flashless" smokeless propellant powder with a progressively increasing rate of burning which comprises adding to and thoroughly incorporating with soluble nitrocellulose between from one-half of one per cent to twenty per cent of a flame propagating agent and completely colloiding with ether and alcohol.

4. The process of making "flashless" smokeless propellant powder which comprises adding to and thoroughly incorporating with soluble nitrocellulose a relatively small proportion of black powder and afterward colloiding with ether and alcohol.

5. The process of making flashless smokeless propellant powder which comprises adding to soluble nitrocellulose a small proportion of black powder, intimately incorporating said nitrocellulose and said black powder, and then colloiding the nitrocellulose with a suitable solvent.

6. The process of making flashless explosive powder with a progressively increasing rate of burning which comprises so mixing soluble nitrocellulose with a relatively

rapid burning flame propagating agent and a nitrocellulose colloiding agent that the action of the colloiding agent will take place substantially after distribution of the flame propagating agent throughout the nitrocellulose, completely colloiding and forming the colloided nitrocellulose into grains, whereby the colloided cellulose grains will be intercellularly impenetrated with the flame propagating agent and the rapid combustion of the latter will carry the flame rapidly from the exposed surfaces into the interior of the grains and effect a relatively early complete consumption of the powder.

7. The process of making flashless explosive powder which comprises so mixing soluble nitrocellulose with black powder and a nitrocellulose colloiding agent that the action of the colloiding agent will take place substantially after distribution of the black powder throughout the nitrocellulose, and forming the colloided nitrocellulose into grains, whereby the colloided cellulose grains will be intercellularly impenetrated with the black powder and the rapid combustion of the latter will carry the flame rapidly from the exposed surfaces into the interior of the grains and effect a relatively early complete consumption of the powder.

8. The process of making flashless smokeless propellant powder with a progressively increasing rate of burning which comprises adding to and thoroughly incorporating with soluble nitrocellulose a flame propagating agent, together with ether and alcohol, completely colloiding and retaining the flame propagating agent in the colloided finished explosive.

9. The process of making flashless smokeless propellant powder with a progressively increasing rate of burning which comprises adding to and thoroughly incorporating with soluble nitrocellulose between from one-half to one per cent to twenty per cent of a flame propagating agent together with ether and alcohol and completely colloiding to produce a powder containing such agent in distributed form.

10. The process of making flashless smokeless propellant powder which comprises adding to and thoroughly incorporating with soluble nitrocellulose a relatively small proportion of black powder together with ether and alcohol.

11. The process of making flashless smokeless propellant powder with a progressively increasing rate of burning which comprises adding to nitrocellulose a small proportion of an agent adapted to give a relatively quick local combustion, and intimately incorporating said nitrocellulose with said agent and completely colloiding the nitrocellulose by a suitable solvent.

12. The process of making flashless smokeless propellant powder which comprises add-

ing to soluble nitrocellulose a small proportion of black powder, and intimately incorporating said nitrocellulose and said black powder together with a suitable solvent.

5 13. A "flashless" smokeless propellant powder with a progressively increasing rate of burning, which comprises at least eighty per cent of completely colloided nitrocellulose containing approximately one-half of 10 one per cent to twenty per cent of a flame propagating agent thoroughly distributed throughout the mass of the nitrocellulose.

14. A "flashless" smokeless propellant powder which comprises at least eighty per 15 cent of colloided nitrocellulose containing a relatively small proportion of black powder distributed throughout the mass of the nitrocellulose.

15. A propellant explosive containing 20 black powder and nitrocellulose intimately blended with each other, the nitrocellulose being present in preponderating proportion.

16. A propellant explosive containing 25 black powder and nitrocellulose intimately blended with each other, the nitrocellulose being present in preponderating proportion and as an integral mass.

17. As a flashless smokeless powder with a progressively increasing rate of burning, 30 an integral cellular body of completely col-

loided nitrocellulose carrying a flame propagating agent within its cells.

18. A perforated smokeless and flashless powder consisting of cellular integral bodies of colloided nitrocellulose carrying a 35 flame propagating agent within its cells.

19. As a new type of flashless smokeless propellant powder, perforated bodies of relatively slow burning colloided nitrocellulose, said bodies being cellular and containing solids within the cells adapted for quick 40 disappearance during combustion with production of open cavities.

20. As a new flashless smokeless propellant, a perforated powder grain of colloided 45 nitrocellulose, said grain being of honeycomb structure and containing a flame propagating solid within the cells of the honeycomb.

21. As a new flashless smokeless propellant, a perforated powder grain of colloided nitrocellulose, said grain being of honeycomb structure and containing black powder 50 within the cells of the honeycomb.

In testimony of which invention, we have 55 hereunto set our hands, at Wilmington, Delaware, on this 22nd day of April, 1920.

FRANCIS I. DU PONT.  
ERNEST DU PONT.